

Aug. 7, 1928.

**1,680,045**

V. O. HOMERBERG ET AL.

## METHOD OF TREATING COPPER ALLOYS AND IMPROVED PRODUCT

Filed Jan 28 1926

2 Sheets-Sheet 1

Fig. 1.



40 50 60 70 80 90 100  
Inventors, *Victor O. Hamerberg*,  
*Dexter N. Shaw*,  
by their Attorneys *Hanson, Hanson*

Aug. 7, 1928.

1,680,045

V. O. HOMERBERG ET AL

METHOD OF TREATING COPPER ALLOYS AND IMPROVED PRODUCT

Filed Jan. 28, 1926

2 Sheets-Sheet 2

FIG. 2



Inventors:

Victor O. Homerberg,  
Dexter N. Shaw,  
by their Attorneys,  
Hawson & Hawson.

Patented Aug. 7, 1928.

1,680,045

# UNITED STATES PATENT OFFICE.

VICTOR O. HOMERBERG, OF BELMONT, MASSACHUSETTS, AND DEXTER N. SHAW, OF PHILADELPHIA, PENNSYLVANIA.

## METHOD OF TREATING COPPER ALLOYS AND IMPROVED PRODUCT.

Application filed January 28, 1926. Serial No. 84,386.

We have discovered a method of treating copper alloys, whereby it becomes possible to obtain products having definite predetermined characteristics of tensile strength, 5 hardness or ductility, according to the result desired. The characteristic feature of our method is a double heat treatment with intermediate quenching, the first heat treatment being at a relatively high temperature, while the temperature of the second heat treatment is lower, but will vary with the characteristics desired in the finished product. Our process has been found particularly valuable for the heat treatment of 10 brass such as 60-40 brass or Muntz metal, but it may also be applied to other brasses, ranging from 63% to 45% copper, and it may also be applied to other copper alloys, of which the temperature composition diagram 15 resembles that portion of the brass diagram where Muntz metal is found. Portions of both the copper-tin (bronze) and copper-aluminum diagrams have such resemblances. 20 One accepted copper-zinc temperature-composition diagram is shown diagrammatically in Fig. 1. The exact points of this curve are at the present time in controversy, hence this diagram is merely illustrative and 25 not to be considered theoretically correct. The portion of the curve to which this invention applies is approximately between 37 and 55% zinc. The portion bounded by AD and BC is known as the beta field and is a 30 single solid solution which exists in equilibrium at points above the critical temperature shown by the lines AD and BC. If an alloy in the form of the single solid solution, beta, is rapidly cooled, the beta will be obtained 35 at room temperature. Upon reheating, at temperatures disclosed, the beta will be transformed into the structure in equilibrium at the reheating temperature. For each 40 reheating temperature, there is a corresponding crystalline structure and corresponding physical properties. The relation of the 45 physical properties to the reheating temperature is illustrated in Fig. 2 and will be considered below. 50 There may be present small percentages up to 10% or even more of other metals, such as lead, zinc, tin, aluminum, manganese, iron, nickel, cobalt, chromium, magnesium, tungsten, or non-metallic elements such as arsenic, phosphorus, sulphur. When these ma-

terials are added intentionally, it is for the purpose of improving the properties of the alloy.

The metal to be treated according to our invention may originally have been cast, 60 rolled, drawn, extruded or spun and it may or may not have been previously annealed.

The important thing is that our first heat treatment is at such a relatively high temperature as to be above the critical temperature 65 at which the single solid solution exists. Those alloys to which our invention is applicable normally exist at room temperature made up of two components, usually two 70 solid solutions designated as alpha and beta. The alloys have the further property of transforming into a single solid solution called beta above a certain definite point called the critical temperature. If the alloy is allowed to transform into the beta condition 75 and then is quenched quickly, substantially a single solid solution, beta, will be obtained at room temperature. In 60-40 brass, for example, the critical temperature is 775° C., or thereabouts, but it varies with 80 in limits for different alloys and for different compositions of copper alloys. Thus in an alloy with 52% copper, the temperature might be as low as 550° C. For copper aluminum alloys, the temperatures will vary 85 from 550° C. to 1050° C. This temperature of the critical range is dependent on the composition and can be ascertained from the known diagram.

In practice, we have found a temperature 90 of 825° C. for a period of two hours to be suitable for this first heat treatment in the case of Muntz metal, but as the result at the end of this first treatment is in some measure a function of time and temperature, 95 the latter may be varied somewhat by varying the length of this treatment.

This first heat treatment is followed by a quick quenching, preferably in cold brine, but other quenching media may be 100 used.

The metal will now be in a condition of beta microstructure as the result of rapid cooling, although alpha may be found as a fringe at the grain boundaries. A second heat treatment at temperatures which we have determined will give a product having predetermined characteristics of strength, hardness or ductility. To start with the metal in the beta condition insures that results

which are predetermined and reproducible will be obtained when the metal undergoes the second heat treatment. Heretofore, the properties of the alloy have been dependent 5 on the condition of each piece and no definite heat treatment scheme or schedule has been possible.

For example, let us suppose that we wish to obtain a 60-40 brass of great tensile strength 10 and hardness. We proceed as follows:

Let us assume that the alloy is about 60 parts copper to about 40 parts of zinc, and containing, it may be also quite small percentages of other materials, such as lead, 15 iron or manganese. We first subject this alloy to a temperature of over 775° C. for a length of time which may vary from half an hour to two hours. For example, we have found that a temperature as high as 20 825° C. and a period of treatment as long as two hours have given good results. These factors, temperature and time, may vary, the object being to heat for a time and at a temperature which will transform the alloy into 25 substantially a single solid solution.

At the end of this first heat treatment, the metal is subjected to a quick quenching. Brine at a temperature of -8° C. may be used as the quenching medium. Any other 30 medium will serve which will cause the piece to cool quickly enough to produce substantially pure beta solid solution at room temperature. The metal is now subjected to a second heat treatment, which is below that 35 of the first heat treatment. In practice, we have found that the best results for high tensile strength are obtained when the second heat treatment is somewhere in the neighborhood of 250° C. The piece is kept 40 at this reheating temperature until the single solid solution beta is transformed into alpha plus beta. This usually requires a shorter time than the primary heating. We have obtained good results with a temperature of 45 about 250° C. for this second heat treatment and the length of the treatment half an hour. Thereafter for the production of high tensile strength and hardness the alloy metal 50 is cooled in any convenient way, for we have found that the rate of this final cooling has no appreciable effect on the physical properties of the metal. This treatment will give an alloy which will be free from internal strains, a condition heretofore unknown with 55 a brass of high tensile strength and hardness.

By the described process of double heat treatment, we have obtained the copper alloy, 60-40 brass, with the remarkably high 60 tensile strength of 82,750 pounds per square inch, with no elongation and a hardness of 240 (Brinell at 3000 kg.). The structure when examined microscopically was found to be made up probably of very fine alpha 65 and beta crystals uniformly distributed.

If it is desirable to obtain an alloy having an appreciable elongation but with a high tensile strength and hardness, a reheating temperature of 300° C. or of 350° C. may be used. The exact reheating temperature to 70 be used to obtain the physical properties desired is ascertainable from the predetermined schedule or plot.

Attention is called to our co-pending application Serial No. 689,504, filed January 75 30, 1924, of which the present case is a continuation in part. In our co-pending case, the heat treatment to obtain alloys of high tensile strength and hardness is specifically 80 claimed. There are also product claims directed to new copper alloys of high tensile strength and hardness. In the present case, the claims cover the whole range of reheating temperatures and there are also specific 85 claims for the heat treatment to obtain alloys of high ductility.

If on the other hand, it be desired to obtain an alloy having a high ductility, the reheating temperature used is somewhat higher, that is, from 400° C. or 450° C. to 90 700° C. or to 750° C. depending upon the other physical characteristics accompanying the ductility that are desired.

For example, let us suppose that we wish to obtain a 60-40 brass of high ductility, we 95 proceed as follows:

Let us assume that the alloy is about 60 parts copper to about 40 parts of zinc, and containing, it may be also quite small percentages, other materials, such as lead, iron 100 or manganese. We first subject this alloy to a temperature of over 775° C. for a length of time which may vary from half an hour to two hours. For example, we have found that a temperature as high as 825° C. and a 105 period of treatment as long as two hours have given good results. These factors, temperature and time, may vary, the object being to heat for a time and at a temperature which will transform the alloy into substantially a single solid solution.

At the end of this first heat treatment, the metal is subjected to a quick quenching. Brine at a temperature of -8° C. may be used as the quenching medium. Any other 115 medium will serve which will cause the piece to cool quickly enough to produce substantially pure beta solid solution at room temperature. The metal is now subjected to a second heat treatment, which is below that 120 of the first heat treatment.

In practice, we have found that the best results for high ductility are obtained when the second heat treatment is somewhere in the neighborhood of 450° C. The piece is 125 kept at this reheating temperature until the single solid solution beta is transformed into alpha or the proportions of components, alpha and beta, which are in equilibrium at the reheating temperature.

This usually requires a shorter time than the primary heating. We have obtained good results with a temperature of 450° C. or thereabouts for this second heat treatment 5 and the length of the treatment, half an hour. Thereafter the piece is cooled in any convenient way which will maintain the equilibrium structure at room temperature. Cold water, oil or brine may be used. Treatment 10 of alloys according to the process of the invention gives alloys free from internal strains.

If it be desired to obtain an alloy with a higher tensile strength and hardness than 15 results when a reheating temperature of 450° C. is used, the piece may be heated at temperatures up to the critical temperature, the exact temperature depending on the physical properties desired and being determined 20 from a predetermined schedule, as hereinbefore discussed.

At each reheating temperature, there is an equilibrium microstructure dependent upon the reheating temperature. This is obtained 25 at room temperature by cooling at a rate which will not permit the structure to change. At relatively low temperatures, say below 450° C., the piece may be cooled in the air without a change in the structure 30 taking place. At higher temperatures, it may be necessary to quench the piece in order that the rate of cooling will be sufficiently rapid to obtain the structure of the reheating temperature at room temperature. The 35 physical properties obtained in a given piece are dependent upon the microstructure. As has hereinbefore been mentioned, the very fine uniformly distributed alpha plus beta gives an alloy with remarkable tensile 40 strength and hardness while the alloy obtained at 450° C. has a high elongation with a good tensile strength and hardness.

The following table which is graphically 45 illustrated in the diagrammatic Fig. 2 of the accompanying drawings will serve as a guide to obtain any desired useful character of final product, although the temperature in any given case may be varied slightly, especially if the normal period of half an 50 hour for the second heat treatment be varied:

Table.

| Reheating temperature<br>degrees C. | Brinell hardness |          | Tensile<br>strength,<br>lbs.<br>sq.in. | Per cent<br>elonga-<br>tion<br>in 2 in. |
|-------------------------------------|------------------|----------|----------------------------------------|-----------------------------------------|
|                                     | 500 kg.          | 3000 kg. |                                        |                                         |
| 50° C.                              | 97               | 126      | 35,000                                 | 4.0                                     |
| 150                                 | 100              | 123      | 38,750                                 | 3.0                                     |
| 200                                 | 136              | 149      | 52,500                                 | 1.0                                     |
| 250                                 |                  | 241      | 82,750                                 | 0                                       |
| 300                                 |                  | 163      | 71,250                                 | 9.0                                     |
| 350                                 | 130              | 131      | 65,000                                 | 19.0                                    |
| 400                                 | 119              | 111      | 61,250                                 | 22.0                                    |
| 450                                 | 69               | 68       | 48,750                                 | 55.5                                    |
| 500                                 | 74               | 82.5     | 50,000                                 | 49.0                                    |
| 550                                 | 74               | 85.5     | 55,000                                 | 47.0                                    |
| 600                                 | 76               | 87.1     | 55,000                                 | 47.0                                    |
| 650                                 | 79               | 88.7     | 56,750                                 | 42.5                                    |
| 700                                 | 85               | 88.7     | 55,750                                 | 34.0                                    |
| 750                                 | 96               | 107      | 57,000                                 | 24.5                                    |

From this, it is seen that with a given alloy, it becomes possible to obtain by our double heat treatment a product with almost any desired physical properties from a low tensile piece with high elongation to one 70 having high tensile strength with practically no elongation. These results are definite and can be predetermined by employing the appropriate reheating temperatures.

The figures in the accompanying table and drawing vary with the time and temperatures of operation, and the composition of the alloys being treated and are to be interpreted only as examples of the broad scope 75 of the invention. Considerable modification 80 in these factors is possible with no departure from the essential features of the invention.

We claim:

1. The process of treating those copper 85 alloys whose composition is such that the particular alloy being treated falls within that portion of the temperature-composition diagram of its system which resembles the portion of the copper-zinc temperature-composition diagram in which 60-40 brass 90 is found, which comprises heating the alloy above the critical temperature to obtain substantially a single solid solution; quenching to obtain this substantially single solid solution at room temperature; and thereafter 95 selecting a predetermined reheating temperature corresponding to the physical properties desired, heating at said chosen temperature and subsequently cooling to obtain substantially the structure corresponding 100 to that of the reheating temperature at room temperature.

2. The process of treating brass whose 105 composition is such that the particular alloy being treated falls within that portion of the copper-zinc temperature-composition diagram in which 60-40 brass is found, which comprises heating the alloy above the critical temperature to obtain substantially a single solid solution; quenching to obtain 110 this substantially single solid solution at room temperature; and thereafter selecting a predetermined reheating temperature corresponding to the physical properties desired, heating at said chosen temperature 115 and subsequently cooling to obtain substantially the structure corresponding to that of the reheating temperature at room temperature.

3. The process of treating those copper 120 alloys whose composition is such that the particular alloy being treated falls within that portion of the temperature-composition diagram of its system which resembles the portion of the copper-zinc temperature-composition diagram in which 60-40 brass 125 is found, which comprises heating the alloy to a point above its critical temperature to obtain substantially a single solid solution; quenching to obtain substantially a single 130

solid solution at room temperature; reheating at a temperature which will give a structure corresponding to the properties desired; and thereafter cooling to obtain substantially this structure at room temperature.

4. The process of treating brass whose composition is such that the particular alloy being treated falls within that portion of the copper-zinc temperature-composition diagram in which 60-40 brass is found, which comprises heating the alloy to a point above its critical temperature to obtain substantially a single solid solution; quenching to obtain substantially a single solid solution at room temperature; reheating at a temperature which will give a structure corresponding to the properties desired and thereafter cooling to obtain substantially this structure at room temperature.

5. The process of treating those copper alloys whose composition is such that the particular alloy being treated falls within that portion of the temperature-composition diagram of its system which resembles the portion of the copper-zinc temperature-composition diagram in which 60-40 brass is found, which comprises heating the piece above the critical temperature to obtain substantially a single solid solution; quenching quickly to obtain substantially a single solid solution at room temperature; reheating the piece according to a predetermined schedule in order to obtain predetermined physical properties; and thereafter cooling to obtain substantially the structure corresponding thereto at room temperature.

6. The process of treating brass whose composition is such that the particular alloy being treated falls within that portion of the copper-zinc temperature-composition diagram in which 60-40 brass is found, which comprises heating the piece above the critical temperature to obtain substantially a single solid solution; quenching quickly to obtain substantially a single solid solution at room temperature; reheating the piece according to a predetermined schedule in order to obtain predetermined physical properties; and thereafter cooling to obtain substantially the structure corresponding thereto at room temperature.

7. The process of treating those copper alloys whose composition is such that the particular alloy being treated falls within that portion of the temperature-composition diagram of its system which resembles the portion of the copper-zinc temperature-composition diagram in which 60-40 brass is found, which comprises subjecting the alloy to a heat treatment above its critical temperature to obtain substantially a single solid solution, followed by quick quenching; and then to a second heat treatment at a lower temperature, followed by cooling at a rate which will give substantially the structure of the reheating temperature at room temperature.

a rate which will give substantially the structure of the reheating temperature at room temperature.

8. The process of treating brass whose composition is such that the particular alloy being treated falls within that portion of the copper-zinc temperature-composition diagram in which 60-40 brass is found, which comprises subjecting the alloy to a heat treatment above its critical temperature to obtain substantially a single solid solution, followed by quick quenching; and then to a second heat treatment at a lower temperature, followed by cooling at a rate which will give substantially the structure of the reheating temperature at room temperature.

9. The process of treating brass whose composition is such that the particular alloy being treated falls within that portion of the copper-zinc temperature-composition diagram in which 60-40 brass is found, which comprises subjecting the alloy to a heat treatment above  $775^{\circ}$  C. to obtain substantially a single solid solution, followed by quick quenching; and then to a second heat treatment at a lower temperature, followed by cooling at a rate which will give substantially the structure of the reheating temperature at room temperature.

10. The process of treating copper alloys whose composition is such that the particular alloy being treated falls within that portion of the temperature-composition diagram of its system which resembles the portion of the copper-zinc temperature-composition diagram in which 60-40 brass is found and which alloy is made up of substantially a single solid solution which comprises heating the alloy at a temperature below the critical temperature to cause a crystalline transformation of the single solid solution into two solid solutions; and thereafter cooling to obtain substantially the structure corresponding to the reheating temperature at room temperature.

11. The process of treating brass whose composition is such that the particular alloy being treated falls within that portion of the copper-zinc temperature-composition diagram in which 60-40 brass is found and which alloy is made up of substantially a single solid solution, which comprises heating the alloy at a temperature below the critical temperature to cause crystalline transformation of the single solid solution into two solid solutions; and thereafter cooling to obtain substantially the structure corresponding to the reheating temperature at room temperature.

12. The process of treating brass whose composition is such that the particular alloy being treated falls within that portion of the copper-zinc temperature-composition diagram in which 60-40 brass is found, which comprises heating the alloy above the criti-

cal temperature to form substantially a single solid solution; quenching quickly to obtain substantially a single solid solution at room temperature; reheating at a temperature between 400° C. and 750° C.; and thereafter cooling to obtain substantially the structure corresponding to that of the reheating temperature at room temperature, whereby an alloy of high ductility is obtained.

13. The process of treating brass whose composition is such that the particular alloy being treated falls within that portion of the copper-zinc temperature-composition diagram in which 60-40 brass is found, which comprises heating the alloy above the critical temperature to form substantially a single solid solution; quenching quickly to obtain substantially a single solid solution at room temperature; reheating at a temperature in the neighborhood of 450° C.; and thereafter cooling to obtain substantially the structure corresponding to that of the reheating temperature at room temperature, whereby an alloy of high ductility is obtained.

14. The process of treating brass whose copper content is approximately 60%, which comprises heating the alloy above the critical temperature to form substantially a single solid solution; quenching quickly to obtain substantially a single solid solution at room temperature; reheating at a temperature between 400° C. and 750° C.; and thereafter quenching to obtain substantially the structure corresponding to that of the reheating temperature at room temperature, whereby an alloy of high ductility is obtained.

15. The process of treating brass whose copper content is approximately 60%, which comprises heating the alloy above the critical temperature to form substantially a single solid solution; quenching quickly to obtain substantially a single solid solution at room temperature; reheating at a temperature in the neighborhood of 450° C.; and thereafter quenching to obtain substantially the structure corresponding to that of the reheating temperature at room temperature, whereby an alloy of high ductility is obtained.

16. The process of treating brass whose copper content is approximately 60%, made up of substantially a single solid solution, which comprises heating the alloy at a temperature between 400° C. and 750° C.; and thereafter cooling to obtain substantially the structure corresponding to the reheating temperature at room temperature, whereby an alloy of high ductility is obtained.

17. The process of treating brass whose copper content is approximately 60%, made up of substantially a single solid solution, which comprises heating the alloy to a temperature in the neighborhood of 450° C.; and thereafter cooling to obtain substantially the structure corresponding to the reheating temperature at room temperature, whereby an alloy of high ductility is obtained.

18. The process of treating those copper alloys whose composition is such that the particular alloy being treated falls within that portion of the temperature-composition diagram of its system which resembles the portion of the copper-zinc temperature-composition diagram in which 60-40 brass is found, which comprises subjecting the alloy to a heat treatment above its critical temperature to obtain substantially a single solid solution; quenching at a rate which will insure substantially a single solid solution at room temperature; and thereafter reheating the piece at a temperature below its critical temperature.

19. The process of treating brass whose composition is such that the particular alloy being treated falls within that portion of the copper-zinc temperature-composition diagram in which 60-40 brass is found, which comprises subjecting the alloy to a heat treatment above its critical temperature to obtain substantially a single solid solution; quenching at a rate which will insure substantially a single solid solution at room temperature; and thereafter reheating the piece at a temperature below its critical temperature.

20. The process of treating brass whose copper content is approximately 60%, which comprises heating the alloy above the critical temperature to form substantially a single solid solution; quenching quickly to obtain substantially a single solid solution at room temperature; and thereafter reheating the piece at a temperature between 400° C. and 750° C., whereby an alloy of high ductility is obtained.

21. The process of treating brass whose copper content is approximately 60%, which comprises heating the alloy above the critical temperature to form substantially a single solid solution; quenching quickly to obtain substantially a single solid solution at room temperature; and thereafter reheating at a temperature in the neighborhood of 450° C., whereby an alloy of high ductility is obtained.

VICTOR O. HOMERBERG.  
DEXTER N. SHAW.